

~~TS24/77~~

X 524/8

X 524/526

Ans I.

Nov. 24, 1931.

F. K. HADLEY

1,833,287

COMPOSITION FOR LIFTING FRICTION SKIN IMPRINTS

Filed Sept. 1, 1928



Fig. 1.



Fig. 2.

Inventor:

Frank K. Hadley,  
By Hugh K. Wagner,

Attorney.

## UNITED STATES PATENT OFFICE

FRANK K. HADLEY, OF ST. LOUIS, MISSOURI, ASSIGNOR TO ST. LOUIS RUBBER CEMENT COMPANY, OF ST. LOUIS, MISSOURI, A CORPORATION OF MISSOURI

## COMPOSITION FOR LIFTING FRICTION SKIN IMPRINTS

Application filed September 1, 1928. Serial No. 303,388.

This invention relates to a composition of matter for lifting friction-skin impressions, such as fingerprints, palm prints, sole prints and the like. Fingerprints, as is well known, 5 are impressions from the terminal phalange of the fingers or thumbs, valuable in the identification of individuals because of the fact that their lines, which delineate the ridge configuration of the friction-skin in all its minutiae, 10 vary in each individual from all others. It is also well known that this method of identification of persons is practiced extensively by police operators on account of the certainty of its results in identifying criminals. A 15 criminal may unknowingly leave a print of his fingers on some article or weapon that he has touched, and this print may be too faint to be detected until it is brought out more distinctly, which is usually done by sprinkling 20 thereon or applying thereto by means of an aspirator a finely divided powder, such as bronze or aluminum, that adheres to the faint markings and renders them easily visible by reason of its high lustre or contrast with the 25 color of the surface that is the site of the print. However, fingerprints are often left on surfaces of objects that cannot be removed, and, prior to this invention, the only way to retain a print situated on such an object was 30 to photograph the print after it had been developed by powdering it. Much difficulty, however, is experienced in photographing a fingerprint on a curved surface, such as the neck of bottle that may have been used as a 35 weapon, or on a site that is not accessible to a camera, or fingerprints left in places that can not be properly lighted for taking photographs; and, even when photographs are taken under such conditions, they are not 40 always reliable.

Accordingly, the principal purpose of the present invention is the provision of a composition of matter that may be applied to friction skin imprints on divers surfaces, and 45 which, upon withdrawal from such surfaces, will lift the imprint therefrom.

Other objects and advantages, more or less ancillary to the foregoing, will appear in the course of the following description of an 50 illustrative embodiment of the invention.

In the accompanying drawings forming part of this specification, in which like numbers of reference denote like parts wherever they occur,

Figure 1 is a plan view, with parts broken 55 away, of the means for utilizing the composition of this invention; and

Figure 2 is a transverse sectional view of the same, the thickness being exaggerated for the sake of clearness.

Briefly described, the composition of the invention provides a body having a surface which is sufficiently pliable to conform intimately to the surface on which the powdered imprint is situated, which is sufficiently adhesive to retain on its conforming surface the powder to which it is applied, and yet is not liable to adhere so strongly to the imprint-bearing surface to which it is applied as to prevent its being pulled away therefrom intact. Preferably a protective covering is detachably applied to the powder-or-imprint-retentive surface of the body.

The composition is best used in connection with a flexible base, preferably finely woven 75 fabric 1, having a coating 2 of the composition applied to one side thereof, and a cover sheet 3, preferably of celluloid or other transparent flexible sheeting, impressed on the coating 2. In order to present a finger print 80 or other friction-skin imprint most conspicuously, the coating 2 should be of a color that forms a strongly contrasting background for the color of the powder, and to this end black is deemed preferable. The fabric is also 85 preferably of the same color, in order to intensify or deepen the color of the coating 2, since the color of the fabric might be faintly visible through the coating 2, especially if the latter is very thin.

The coating 2 is a composition of matter that preferably comprises a rubber base and a quantity of binding and softening material sufficient to give the composition a consistency 95 that will render it sufficiently pliable to follow intimately the surface of the body or object from which the friction-skin impression is to be removed, and sufficiently adhesive to lift the powder of the impression from the impression-imparting surface, but not adhe- 100

sive to such a degree as to prevent the composition from being withdrawn intact from the impression-imparting surface. The composition may also contain suitable coloring matter. In preparing the composition it is preferable to use Crepe and Guayule rubber as a base, Cumar R. S. (rubber soft) as a binder, cottonseed oil and petrolatum as softeners, and carbon black as coloring matter.

10 The best results may be obtained when these ingredients are in the following proportions by weight: Crepe rubber, twenty-five parts; Guayule rubber, eight and one-fourth parts; carbon black, one-eighth part; Cumar rubber soft, three and one-half parts; cottonseed oil, two parts; and petrolatum, one part.

15 The rubber is first weighed and thoroughly broken down by the rolls of a mixer. The various other ingredients of this formula are weighed and mixed in a receptacle, and are then added to the broken down rubber in the mixer, in which these other ingredients are thoroughly mixed with the rubber.

20 The prepared compound is then run on a "calender" machine and impressed on one side of the black woven fabric sheeting that forms the base 1. The weaving of the fabric 1 is sufficiently close and fine to prevent the composition from being forced through the 25 interstices of the fabric to the opposite side, while at the same time permitting the composition to become thoroughly imbedded in the interstices adjacent to the coated side of the fabric 1, thereby firmly uniting the fabric 30 1 and the coating 2. After this operation, the coated sheeting is then cut to the size of the celluloid sheeting that is to cover the coating 2. The celluloid 3 is then pressed against the coat 2 of the coated sheet in a machine 35 known to the art as a "doubler", which forces out all the air which may intervene between the celluloid 3 and the coat 2. The finished material is then ready for use, the celluloid 40 adhering detachably to the coating 2.

45 In lifting a finger print, or in fact a print of the foot or any part of the human body, by means of a sheet coated with the composition of this invention, a piece of the sheet sufficiently large to cover the imprint is cut 50 from the prepared sheet, reserving the residue for future use. The usual powdering process is then employed to develop the impression, wherever it may be, whether on metal, wood, glass, or on any smooth surface. The 55 celluloid covering of the piece of sheet material is then lifted from the coating underneath and the coated side of the cut piece is impressed against the powdered imprint, and the imprint adheres to the coated side 60 and is lifted off perfectly with it from the surface to which it has been applied when the cut piece is pulled away from said surface. The lifted celluloid is then replaced on the cut piece to protect the impression 65 retained on the coating thereunder, thereby

enabling the print to be preserved for future use. The celluloid being transparent, the print is visible and may also be photographed for distribution without lifting the celluloid cover sheet 3 from the coating 2.

70 The finger print lifting material of this invention can also be used in hospitals for preserving the imprint of babies' feet or hands, by first placing feet or hands on a proper sized glass plate and then taking the imprint from the glass in the same manner 75 as described above. Another method of taking an impression from the body consists in powdering the glass, then pressing the foot or other portion of the body on the glass, and subsequently pressing such portion of the body on the imprint-receptive material of 80 this invention, which will leave a perfect print thereon, the ridges of the skin receiving the powder from the glass and transferring it to the contiguous surface of the composition 2.

85 The flexibility of the sheet of lifting material enables it to be applied to curved and irregular surfaces.

90 Having thus fully described this invention, I hereby reserve the benefit of all changes in form, arrangement, order, or use of parts, as it is evident that many minor changes may be made therein without departing from the spirit of this invention or 95 the scope of the following claims.

I claim:

1. A composition for lifting friction-skin 100 imprints, comprising substantially by weight twenty-five parts of Crepe rubber, ten parts of Guayule rubber, one-eighth part of carbon black, three parts of Cumar soft rubber, two parts of cottonseed oil, and one and one-half parts of pine tar.

2. A composition for lifting friction-skin 105 imprints, comprising a rubber base and a quantity of soft rubber and cottonseed oil sufficient to give the composition a consistency that will render it sufficiently pliable to follow intimately the surface of the object from which the friction-skin impression is to be removed and sufficiently adhesive to lift the powder of the impression from the impression-imparting surface.

3. A composition for lifting friction-skin 110 imprints comprising Crepe and Guayule rubber, Cumar soft rubber, cottonseed oil and a coloring agent.

4. A composition for lifting friction-skin 115 imprints comprising Crepe and Guayule rubber, Cumar soft rubber, pine tar and a coloring agent.

In testimony whereof I hereunto affix my signature.

FRANK K. HADLEY.

125

130